

1

2,996,453

LUBRICATING OIL COMPOSITION

Louise F. Peale, Philadelphia, and Joseph F. Messina, Havertown, Pa., assignors to the United States of America as represented by the Secretary of the Army  
No Drawing. Filed Mar. 30, 1960, Ser. No. 18,779

1 Claim. (Cl. 252—49.8)

(Granted under Title 35, U.S. Code (1952), sec. 266)

The invention described herein may be manufactured and used by or for the Government for governmental purposes without the payment to us of any royalty thereon.

This invention relates to the art of lubrication and more particularly concerns a lubricity additive to both synthetic and mineral lubricating oils to provide improved extreme pressure, anti-wear and anti-friction properties thereto.

As is well known to those familiar with the art, during the past decade or so, machine design has involved the use of smaller gears of the worm and hypoid type which operate under extremely high pressure loads. Consequently, for effective lubricating, lubricants capable of withstanding pressures appreciably higher than those of which ordinary synthetic or mineral type lubricating oil films will rupture have been required.

The ever-increasing demand for extreme pressure lubricants has led to the development of various extreme pressure agents and to their proposed incorporation in both synthetic and mineral lubricating oils in amounts sufficient to improve their extreme pressure characteristics. The chemically active type of extreme pressure agents are, as is well known in the art, the most widely used. Presumably, these materials possess the property of reacting chemically with the metal surfaces to be lubricated, under the conditions of operation, to produce thereon films or coatings. These films or coatings are capable either of withstanding by themselves the extreme pressure loads or protecting the relatively moving metal surfaces against seizure and scoring.

In addition to the property of being able to withstand extreme pressure loads, there are other important factors that must be considered in evaluating lubricants for hypoid gear systems and the like. Among the most important are the tendency of the lubricant to wear the surfaces of the relatively moving metal surfaces and to offer unnecessary friction therebetween. Numerous materials have been developed in attempts to meet these requirements satisfactorily. Insofar as is known, however, no single additive compound or lubricity agent to both synthetic and mineral lubricating oils imparting good extreme pressure, anti-wear and anti-friction characteristics to the base oil has been found.

Various phosphorus compounds are currently employed as lubricity additives to base oils of synthetic or mineral type. For example, the presently used triphenyl, tritolyl and oleyl lauryl phosphates improve the extreme pressure characteristics of mineral oils but are deficient in anti-wear improvement.

A commercial compound, tricresyl phosphate, while enhancing anti-wear and anti-friction characteristics to both type oils fails to improve their extreme pressure properties.

It is therefore a principal object of this invention to provide a lubricity additive or agent capable of being incorporated in synthetic or mineral oils and yet imparting good extreme pressure, anti-wear and anti-friction properties thereto.

It is another object of this invention to provide such an additive wherein the starting materials are relatively inexpensive and abundantly available.

2

These and other objects will be apparent as the invention is more fully hereinafter disclosed.

In accordance with these objects it has been discovered that minor additives of a selected long chain phosphate to bis(2-ethylhexyl) sebacate and to various mineral oils is amenable therewith. Further, the blended lubricant is characterized by better than satisfactory extreme pressure, anti-wear and anti-friction properties.

The synthetic lubricating oil chosen for the purposes of this invention is bis(2-ethylhexyl) sebacate. This oil is typical of the synthetic diester base oils.

The mineral oils selected presented in the tables following are SAE 40 and SAE 90. It is to be understood that the invention is not to be considered as being limited to the specific viscosities as it will be apparent to those skilled in the art that a wide variety of viscosities of mineral oils may be employed in formulating the lubricant contemplated herein. The lubricity additive, which in accordance with this invention is blended with the synthetic or mineral oil, comprises a long chain phosphate dibutyl lauroxypropyl phosphate. To date, its use has been generally restricted to low temperature plasticizing for vinyl chloride polymers and the like. Its structural formula is:



and may be prepared in various ways but is, for the most part, conveniently prepared by the following method: 3-hydroxypropyl laurate, having a boiling point of 137° to 145° C. at 0.1 to 0.15 mm. was prepared in 50 to 70% yield by refluxing 80 grams of lauric acid, 305 grams of 1,3-propanediol, 200 ml. of toluene, and 2 grams concentrated sulfuric acid for 4.5 hours with azeotropic removal of water. The reaction product was washed several times with water to remove excess glycol and catalyst, and was then fractionally distilled. 46 grams of dibutyl chlorophosphate was slowly added to a stirred solution of 3-hydroxypropyl laurate, 11.9 grams of pyridine and 150 ml. anhydrous ether. Dibutyl lauroxypropyl phosphate having a boiling point of 169° to 185° C. at 0.13 mm. was obtained in 50% yield as a colorless, odorless liquid.

1 through 6 weight percent of the dibutyl lauroxypropyl phosphate was intimately blended with each of bis(2-ethylhexyl) sebacate and varying SAE mineral oils and then subjected to extreme pressure, anti-wear and anti-friction evaluation tests. These tests were conducted on conventional laboratory equipment and will not be described in detail, as their operations are well known to those skilled in the art. For example, anti-wear data were obtained on the Shell 4-ball wear tester. Extreme pressure data were determined using the well-known Falex and Shell 4-ball extreme pressure tester while anti-friction data were obtained on a modified Bowden and Leben apparatus. The operation of the Shell 4-ball testers, if the reader finds it necessary, may be found amply described in an article by G. D. Boerlage, Engineering, vol. 136 (1933), p. 46 et seq. The Falex extreme pressure tester is described in Lubrication Engineering, September 1946, V. A. Ryan, while the modified Bowden and Leben apparatus appears in The Friction and Lubrication of Solids, F. P. Bowden and D. Tabor, Oxford Clarendon Press, Oxford, England, 1950, pp. 73-74.

For purposes of clarity of illustration, the data obtained in evaluating the aforementioned properties are tabulated separately below.

3  
TABLE I  
Comparative extreme pressure data

| Item No. | Oil                                | Additive                         | Wt. Percent Additive | Falex Extreme Pressure Jaw Load Failure, lbs. | Shell 4-Ball Extreme Pressure |     |
|----------|------------------------------------|----------------------------------|----------------------|-----------------------------------------------|-------------------------------|-----|
|          |                                    |                                  |                      | Seizure Load (Kg.) a                          | Weld Load (Kg.) b             |     |
| 1.       | Bis(2-ethylhexyl) sebacate.        | None                             |                      | 1,000                                         | 50                            | 100 |
| 2.       | do                                 | Dibutyl lauroxypropyl phosphate. | 2                    | 2,000                                         | 90                            | 180 |
| 3.       | do                                 | do                               | 5                    | 1,750                                         | 90                            | 160 |
| 4.       | do                                 | Triisopropyl phosphate.          | 5                    | 1,750                                         | 80                            | 140 |
| 5.       | do                                 | Diisopropyl phosphate.           | 1                    | 1,750                                         | 110                           | 160 |
| 6.       | SAE 40 Mineral oil.                | None                             |                      | 600                                           | 50                            | 140 |
| 7.       | do                                 | Dibutyl lauroxypropyl phosphate. | 2                    | 2,000                                         | 70                            | 160 |
| 8.       | do                                 | do                               | 5                    | 2,750                                         | 120                           | 180 |
| 9.       | do                                 | Commercial tricresyl phosphate.  | 2                    | 600                                           | 60                            | 140 |
| 10.      | do                                 | do                               | 5                    | 600                                           | 60                            | 140 |
| 11.      | SAE 90 Mineral oil.                | None                             |                      | 600                                           | 40                            | 100 |
| 12.      | do                                 | Dibutyl lauroxypropyl phosphate. | 2                    | 1,500                                         | 90                            | 180 |
| 13.      | do                                 | do                               | 5                    | 1,750                                         | 100                           | 180 |
| 14.      | SAE 90 Commercial hypoid gear oil. | do                               | (e)                  | 1,750                                         | 100                           | 180 |

a Seizure may be defined as the load at which a significant increase in wear scar diameter takes place.

b Weld may be defined as the load at which the balls fuse together.

e Unknown.

Item Nos. 4, 5 and 9, triisopropyl and diisopropyl phosphates and tricresyl phosphate are presently used as lubricity agents in diester lubricating oils, such as bis(2-ethylhexyl) sebacate, and the weight percentages shown are believed to be the optimum percentages used commercially.

TABLE II  
Comparative anti-wear data

| Item No. | Oil                                | Additive                         | Wt. Percent Additive | Shell 4-Ball Wear Scar Diameter, mm. |
|----------|------------------------------------|----------------------------------|----------------------|--------------------------------------|
| 1.       | Bis(2-ethylhexyl) sebacate.        | None                             |                      | 0.859                                |
| 2.       | do                                 | Dibutyl lauroxypropyl phosphate. | 2                    | .501                                 |
| 3.       | do                                 | do                               | 5                    | .587                                 |
| 4.       | do                                 | tricresyl phosphate.             | 2                    | .433                                 |
| 5.       | do                                 | do                               | 5                    | .401                                 |
| 6.       | SAE 40 Mineral Oil                 | None                             |                      | .734                                 |
| 7.       | do                                 | Dibutyl lauroxypropyl phosphate. | 2                    | .675                                 |
| 8.       | do                                 | do                               | 5                    | .602                                 |
| 9.       | do                                 | Tricresyl phosphate.             | 2                    | .556                                 |
| 10.      | do                                 | do                               | 5                    | .504                                 |
| 11.      | SAE 90 Mineral oil.                | None                             |                      | .637                                 |
| 12.      | do                                 | Dibutyl lauroxypropyl phosphate. | 2                    | .630                                 |
| 13.      | do                                 | do                               | 5                    | .557                                 |
| 14.      | SAE 90 Commercial hypoid gear oil. | do                               | un-known             | .525                                 |

Item Nos. 4 and 5, tricresyl phosphate, is used extensively as an effective anti-wear agent in both synthetic and mineral oils.

5  
TABLE III  
Comparative coefficient of friction data

| Item No. | Oil                                | Additive                         | Wt. Percent Additive | Coefficient of Friction |
|----------|------------------------------------|----------------------------------|----------------------|-------------------------|
| 10       |                                    |                                  |                      |                         |
| 1.       | None                               | None                             |                      | .45                     |
| 2.       | do                                 | Dibutyl lauroxypropyl phosphate. | 2 and 5              | .04                     |
| 3.       | do                                 | Lauroic acid                     | 2                    | .10                     |
| 4.       | do                                 | Oleic Acid                       | 2                    | .08                     |
| 5.       | do                                 | Stearic Acid                     | 2                    | .05                     |
| 6.       | do                                 | Tricresyl phosphate.             | 2                    | .07                     |
| 7.       | do                                 | Dialkyl acid phosphite.          | 2                    | .06                     |
| 8.       | Bis(2-ethylhexyl) sebacate.        | None                             |                      | .15                     |
| 9.       | do                                 | Dibutyl lauroxypropyl phosphate. | 2                    | .10                     |
| 10.      | do                                 | do                               | 5                    | .14                     |
| 11.      | do                                 | Dialkyl Acid Phosphite.          | 2                    | .10                     |
| 12.      | SAE 90 Mineral Oil                 | None                             |                      | .17                     |
| 13.      | do                                 | Dibutyl lauroxypropyl phosphate. | 2 and 5              | .11                     |
| 14.      | SAE 90 Commercial hypoid gear oil. |                                  |                      | .10                     |
| 30       |                                    |                                  |                      |                         |

Item 14, hypoid gear oil, is a commercial product containing phosphorus, sulfur and chlorine additives. Items 3, 4, 5, 6, 7 and 11 are commercial additives.

35 All values presented in Tables I, II and III above are averages of five different measurements. Maximum variance among the five values was confined to within a 10% range. Although 2 and 5 weight percentages of dibutyl lauroxypropyl phosphate are presented in the 40 tables, it should be understood that intermediate additions were found equally satisfactory, that is, between 2 and 5 weight percentages.

From the data hereinabove set forth, it will become apparent that the lubricity additive of the present invention, when confined within the prescribed range of about 45 2 to 5 weight percentages is positive and specific in improving the extreme pressure, anti-wear and anti-friction characteristics of the base oil. While, in a few instances, the dibutyl lauroxypropyl phosphate did not improve a 50 particular characteristic as markedly as one of the commercial additives, it is believed that no known commercial product to date has been found capable of improving all these requirements in both synthetic and mineral type oils.

We claim:

55 A lubricant composition having improved extreme pressure, anti-wear and anti-friction properties suitable for use in hypoid gear systems, said lubricant composition consisting essentially of about 2 to 5 weight percent of dibutyl lauroxypropyl phosphate and the balance being 60 selected from the group consisting of bis(2-ethylhexyl) sebacate and mineral oil.

References Cited in the file of this patent

UNITED STATES PATENTS

65 2,285,853 Downing et al. June 9, 1942  
2,478,441 Wiley Aug. 9, 1949

FOREIGN PATENTS

70 560,741 Great Britain July 22, 1958

OTHER REFERENCES

Atkins et al.: "Development of Additives and Lubricating Oil Compositions," I. and E. Chem., vol. 39, No. 4, 75 April 1947, pp. 491-497.